

March 3, 1931.

S. H. DAVIS ET AL

1,795,079

METHOD OF ELECTROPLATING ZINC ON IRON OR STEEL

Filed Sept. 12, 1928



INVENTORS

Sidney H. Davis,  
Carl O. Anderson,  
William N. Smith,  
Herbert R. Hanley,

BY *Blount & Sellard*

ATTORNEYS

WITNESS

*F. G. Hartman.*

## UNITED STATES PATENT OFFICE

SIDNEY H. DAVIS AND CARL O. ANDERSON, OF BAXTER SPRINGS, KANSAS, AND WILLIAM N. SMITH, OF PLATTEVILLE, WISCONSIN, AND HERBERT R. HANLEY, OF ROLLA, MISSOURI, ASSIGNORS TO THE CENTURY ZINC COMPANY, A CORPORATION OF OHIO

## METHOD OF ELECTROPLATING ZINC ON IRON OR STEEL

Application filed September 12, 1928. Serial No. 305,429.

The object of our invention, considered in its broadest aspect, is to provide a cyclic method by which zinc from a commercial raw source may be directly plated on an iron or 5 steel article to thereby provide a merchantable article of commerce.

Hitherto the coating of iron or steel articles with zinc has been effected either by the hot dipping process in which the article to be 10 coated is dipped after suitable preparation in a bath of molten spelter, or by the electroplating process in which the deposit of zinc on the article is effected by submerging the latter in a neutral or substantially neutral 15 solution of zinc sulfate or an alkaline solution of cyanide of zinc and then passing an electric current of relatively low density from a soluble zinc anode, likewise submerged in the bath, to the article acting as a cathode. 20 Both of these processes necessarily require initial production from the zinc ore of metallic zinc, either for the preparation of the molten bath or to serve as the soluble anode in the plating bath. When the zinc or spelter 25 is to be used for hot dipping, the most satisfactory results are obtained when the metallic zinc is recovered from the ore by the well known retort process, experiments having shown that the substantially pure metallic 30 zinc derived from the ore by the electrolytic processes now in use is unsatisfactory for hot dipping. In like manner the metallic zinc to be used as the soluble anode in the electroplating process is ordinarily produced by the 35 retort process but irrespective of whether it be produced by the retort process or electrolytically, initial production of the metallic zinc as such is required as a preliminary to its use in the electroplating process, so that 40 in either of the methods hitherto employed for coating iron or steel articles with zinc, the latter must first be produced by one process and then utilized in an entirely separate and different process, i. e., hot dipping or 45 electroplating for coating the article.

In accordance with the preferred practice of our method however, we are able in a single cycle comprising a series of inter-related steps to effect direct transfer of the zinc 50 contained in the raw concentrate or other

zinkiferous material to the article to be plated, thus entirely avoiding the necessity for first producing metallic zinc by one series of operations and then utilizing that zinc to form the coating upon the article in another 55 and separate series of operations.

The preferred practice of our method is thus advantageous in numerous respects, among which may be mentioned marked economy in operating costs; a higher percentage 60 of recovery of zinc from the concentrate than has been usual in the methods of recovery heretofore practised, the loss of zinc by our method being less than one-third of that occurring in the combination of retort recovery and hot dipping now in use; permissible recovery of 65 by-product metals such as cadmium and lead contained in the ore which are now wasted or lost when metallic zinc is recovered by the retort method but which have a present value 70 of several dollars per ton of ore. Moreover, we are able in accordance with our invention to produce upon the article a coating of markedly different and superior characteristics to that which it has been possible to produce 75 either by the hot dipping or electroplating process as heretofore practised.

Other advantages and novel features and characteristics of our invention are herein-after more specifically mentioned or will be 80 apparent to those skilled in the art as a more detailed comprehension thereof is acquired from the following description.

As stated, our method is preferably a cyclic one in which, among other things, zinc calcines derived from raw zinc concentrates and/or other zinkiferous materials are continuously leached with an acid solution supplied from the cell or cells in which the plating of the article is effected, and which for convenience may be termed the operating cells, so as to produce a zinc sulfate solution which, after suitable treatment, is fed in regulated quantity to the plating bath so as to maintain the bath, and in which the article to be coated and acting as the cathode and an insoluble anode are suspended, in a relatively highly acid condition while a current of relatively high density is passed from the anode to the cathode to effect the deposition thereon 100

- of metallic zinc supplied from the bath, as distinguished from a soluble zinc anode as in the ordinary electroplating process. Since the action of the current on the bath results in the generation of a quantity of sulphuric acid chemically equivalent to the quantity of the electrodeposited zinc abstracted from the bath, and as since this volume of sulphuric acid is constantly fed back to the zinc calcine or other source from which the zinc is obtained to thereby form fresh zinc sulfate solution containing a chemically equivalent quantity of zinc which in turn is fed back to the bath, the process is a truly cyclic one, it being only necessary during its operation to continuously supply a sufficient quantity of the zinc calcine or other source of zinc to compensate for the amount of metallic zinc deposited on the ferrous articles.
- 20 In the use of an insoluble anode resides an important and distinguishing difference between our method and the ordinary electroplating processes, enabling us as it does to achieve and satisfactorily utilize plating baths of relatively high acidity and currents of high density. In the ordinary electroplating practice, on the other hand, soluble anodes are employed which prohibit the use of relatively high acid solutions or baths since the same by dissolving the anodes would destroy or materially lower their own acidity. By the use of insoluble anodes, however, this result is obviated, and we are thereby enabled to provide a process in which the acid generated in the operating cell or cells is desirably utilized for dissolving the zinc calcine or other zinc material serving as the source of the zinc which is ultimately plated on the ferrous article by the utilization of high density currents with resulting production, through the use of such currents in connection with high acid solutions, of a coating or plating markedly superior to those which it has been possible to heretofore produce by any method or process with which we are familiar.
- 50 The deposition of zinc from highly acid zinc sulfate solutions on iron or steel articles acting as cathodes is first attended by the evolution and deposition of hydrogen at the article or cathode. After a variable interval of time, the exact length of which differs in accordance with operating conditions and the like, the major evolution of this hydrogen ceases and the cathode is found to be incipiently coated with a thin deposit of zinc but during the formation of this initial or incipient coating while the major evolution of the hydrogen is taking place the current efficiency is relatively low with resultant diminution of operating economy. However, after the formation of the initial coating and cessation of the major evolution of hydrogen, the current efficiency increases and 65 the zinc is deposited more readily.

We have found the major evolution of hydrogen can be checked and an initial or "strike coating" of zinc formed on the article in a given interval of time after it has been rendered properly zinc-receptive by pickling and brushing and/or other surface conditioning in the usual or any suitable way, by the use of a current whose density varies almost directly with the acidity of the solution or electrolyte; thus, for example, if the evolution of hydrogen and initial deposit of zinc can be effected on an iron or steel article having a given type of surface in 30 seconds when using a current density of 100 amperes per sq. ft. of cathode surface and a solution containing 5% sulphuric acid, it is requisite to effect the same result when employing a solution containing 10% sulphuric acid, that is, a solution having twice the acidity of the first solution, to employ a current having a density of substantially 200 amperes per sq. ft. of cathode surface. From this it follows that if iron or steel articles are to be coated with zinc to a thickness sufficient for ordinary commercial uses in a reasonable length of time, it is necessary when utilizing relatively high acid solutions to employ currents of relatively great density necessarily requiring extremely heavy busbars, wiring and other instrumentalities for their transportation with resultant enhancement of the cost of initial installation and maintenance as well as of fixed charges during the life of the plant.

Under certain conditions this may not be found objectionable but in accordance with the preferred practice of our invention we consider it generally more advantageous to effect an initial or strike coating on the iron or steel article by means of a current of very high density and at high efficiency and to then form a subsequent coating by using a current of relatively lower density but with equal efficiency with the result that since the high density current is employed but momentarily it is unnecessary to provide means for transporting and handling it of the same capacity and size as would be the case were the said current employed for the longer interval necessary to form a thicker deposit; additionally, as this practice materially shortens the period during which the evolution of hydrogen takes place in large quantities from the steel or iron article acting as a cathode, the production of an ultimate coating of great perfection and high quality is insured.

The present method is desirably carried out as a cyclic and continuous one and to enable those skilled in the art to readily comprehend and practice the same, we will first proceed to describe one way of performing it where raw zinc concentrates are utilized as the source from which the zinc is derived, reference in this connection being

had to the accompanying drawing showing a flow sheet thereof, the method, however, being capable of modification in many particulars without departing from the spirit 5 and scope of the invention, for example as will hereinafter appear, by the employment of metallic zinc instead of raw zinc concentrates as the source of zinc supply.

Pursuant to the preferred practice of the 10 present method, zinc calcines derived by roasting or other suitable treatment of the raw zinc concentrates are continuously leached with an acid solution derived from the cells in which the articles are plated so 15 as to produce a zinc sulfate solution which, after suitable treatment, is fed in regulated quantity to one or more of said cells so as to maintain the baths therein, in which the said articles acting as the cathodes and in 20 soluble anodes are suspended, in a relatively highly acid condition while a current is being passed therethrough from the anodes to the articles to plate thereon metallic zinc supplied from the baths as distinguished 25 from a soluble zinc anode as in the ordinary electroplating process, at least two of such cells being desirably employed, the first of which for convenience may be termed the "strike-coating cell" and the other or others 30 as the operating cell or cells. Since the action of the current on the bath in each cell results in the generation of sulphuric acid in quantity chemically equivalent to the quantity of zinc plated out of the bath and 35 since as this volume of sulphuric acid is ultimately fed back to the zinc calcines or other source from which the zinc is obtained, to thereby form fresh zinc sulfate solution containing a chemically equivalent quantity 40 of zinc which in turn is fed back to the cells, the process is a truly cyclic one, it being only necessary during its operation to continuously supply a sufficient quantity of the zinc calcines or other zinciferous material to 45 make up for the metallic zinc ultimately abstracted from the operation in the form of coatings on the iron and/or steel articles.

Thus, when employing the raw zinc concentrate, the same may first be roasted in the 50 usual way so as to oxidize the zinc sulphide into zinc oxide and, to some extent, into zinc sulfate which compounds are soluble in dilute sulphuric acid and in water respectively. The zinc calcines produced by the roasting 55 operation are then leached with a dilute solution of sulphuric acid which, as hereinafter explained, is drawn from the cells. Due to the immersion of the iron and steel articles in the plating baths or from other causes, 60 this solution may contain some iron which it is necessary to remove, conveniently by first oxidizing the iron sulfate from the ferrous to the ferric state with some effective and permissible oxidizer, for example, manganese dioxide (hydrated) which is produced

as a by-product from the anodes in the strike and operating cells. Following the addition of the manganese dioxide to the solution, conveniently in the leaching tank, an excess of base, for example, zinc oxide in the form of 70 zinc calcine, is added to the solution, thus neutralizing any residual acid and then, by further addition, causing precipitation of the iron as ferric hydrate or similar insoluble iron compound; should arsenic and/or antimony be present they will be precipitated 75 with the iron. At this point all of the zinc which is soluble is in solution as zinc sulfate in the leaching tank; additionally, relatively small amounts of copper and cadmium and possibly other metals such as nickel and cobalt are also in solution as sulfates, these metals 80 having been leached out of the concentrate.

The contents of the leach tank may then be passed to a suitable classifier which separates the coarser particles from the slime and the former may then be carried through a ball mill or other suitable device to grind them to a slime which is returned to the classifier as shown, these slimes constituting the final 85 state of division of the solids remaining from the leaching operation.

From the classifier the slimes may be directed to a Dorr or other suitable thickener 90 in which a large proportion of the liquid is separated from the solids; the thickened slimes may then be passed to a continuous suction filter where the final separation of the solids from the liquid is effected and the filtrate then merged with the liquid coming 95 from the Dorr thickener.

This solution usually contains, as previously noted, some copper and cadmium in addition to the major metal zinc and these, namely, the copper and cadmium, are next precipitated from the solution in any suitable way, desirably by the addition of zinc dust, and together with any excess of the zinc dust then separated from the solution by means of a filter or the like and should any other impurities such as nickel and cobalt be present in the solution they are removed by any of the standard methods of purification utilized in the electrolytic zinc industry. The solids from the filter may then be subjected to any treatment suitable for recovering the cadmium and/or copper as by-products as well as the zinc dust, this treatment forming no part of the present invention; in this permissible recovery of the cadmium and/or copper and other metals as by-products, however, resides one of the advantages of our method, leading, as it does, to a larger monetary yield from each ton of ore treated than 100 is possible when processes are employed which result in the loss of these by-products, such, for example, as the usual retort process.

The purified zinc sulfate solution delivered 105 from the filter is now ready to be fed to the 110

strike and operating cells, and may for convenience be termed the "primary solution".

While for convenience of description we have herein referred to employment of the usual "single leach" process in the preparation of the primary zinc sulfate solution, it will be understood that, if desired, the "double leach" process may be employed instead and under certain conditions will be preferred, the primary object in either case, of course, being to obtain at the lowest possible cost and in the most convenient way a substantially pure neutral zinc sulfate solution which is to be fed to the strike and operating cells to maintain the desired acidity therein and replace the metallic zinc plated out on the ferrous articles. The manner of producing the neutral zinc sulfate heretofore described does not in itself form any part of the present invention as the same is well known and at present in common use in the electrolytic zinc and lithopone industries.

In accordance with the preferred practice of the present invention the plating on the iron or steel article is effected in two or more steps respectively performed in the strike coating cell with a relatively low acid solution and a current of relatively high density and then in one or more operating cells with a solution of higher acidity and a current of relatively lower density. In this manner, as will hereinafter more fully appear, we are able by the substantially momentary passage of the high density current through the strike cell to very rapidly effect an initial strike coating of zinc upon the article without the evolution of an undue amount of hydrogen and with high current efficiency and, after the formation of this coating to thicken the same to any required degree by transporting the initially coated article to the operating cell or cells and passing therethrough for a longer period a current of relatively lower current density, insoluble anodes, desirably of lead, being employed in both the strike and operating cells.

While the method is in operation the baths in the strike and operating cells are respectively automatically maintained in properly acid condition as will hereinafter appear but must be initially brought to that condition by the addition of the proper amount of sulphuric acid or by passing a current from an insoluble anode to build up the acidity of the solution to a proper operating value. The zinc sulfate solution with which the cells are initially filled may be obtained in any desired way, for example, by forming a sufficient quantity of the primary solution in the manner described but utilizing for the leaching operation necessary therefor a dilute sulphuric acid solution supplied from an external source in suitable quantity instead of from the electrolytic cells as in the cyclic operative performance of the method.

As heretofore stated, the bath in the strike cell is preferably maintained at a considerably lower acidity than the bath in the operating cells; thus, for example, good results are obtained when the bath in the former is maintained at an acidity of 4% to 5%, i. e., 40 to 50 grammes of sulphuric acid per thousand cubic centimeters and the bath in the latter at an acidity of 7½% to 10%, i. e., from 75 to 100 grammes of sulphuric acid per thousand cubic centimeters of solution when strike and operating currents having density, respectively of approximately 150 and 60 amperes per sq. ft. of cathode surface are to be employed. The particular acidity of the two baths, however, is capable of considerable variation both above and below the percentages indicated and will usually be determined in practice by the specific operating conditions present, it being of course appreciated that, within limits, the higher the density of the strike current with relation to the acidity of the bath the more rapid will be the deposition of the strike coating and consequently the shorter interval permitted for the evolution of hydrogen. The addition to the baths of a small amount of some suitable addition agent such as glue is usually found advantageous.

The solution in the strike and operating cells having thus been brought to the desired degree of acidity, the iron or steel article to which the coating is to be applied, having been given a suitable surface conditioning as by immersion in an alkali cleaning solution to effect grease removal, followed by rinsing and by pickling to remove scale, followed by rinsing and brushing again followed by alkali cleaning or electro-alkali cleaning if deemed desirable, is suspended in the solution in the strike coating cell to act as a cathode and a direct current passed thereto through the bath from an insoluble anode also suspended in the solution and desirably of lead. As stated, the density of the strike current will be governed more or less by operating conditions and the like, it being, however, desirable to use a current of as high density as possible within the bounds of economic operation, for example, 150 amperes per sq. ft. of cathode surface, a current of this density being capable with a solution having an acidity of 4% to 5% of depositing a very satisfactory strike coating in approximately one minute. It will therefore be apparent that because of the relatively short time this current is flowing, the busbars and other connections and instrumentalities by which it is carried may, without becoming unduly overloaded and heated, be of materially smaller size and capacity than would be required were the current directed through them for a materially longer interval, with consequent decrease in cost of initial installation, plant maintenance and fixed charges.

As soon as the strike coating is formed, the strike current is shut off and the article being plated transferred to the operating cell containing a bath of zinc sulfate of considerably higher acidity than that in the strike-coating cell and after the article has been immersed therein a direct current of lower density than employed in the strike cell is passed from an insoluble anode, desirably of lead, to the article acting as a cathode for an interval sufficient to form an ultimate plating of the desired thickness on the article. For satisfactory and economical operation, a current having a density of 60 amperes per sq. ft. of cathode surface may be employed with a bath having an acidity of substantially 10%, but as in the case of the strike coating cell the acidity of the bath and the density of the current are capable of considerable variation from these figures, while, of course, the length of time during which the current is passed will be determined by the thickness of the plating it is desired to produce on the article. As a guide, it may be stated that the application of 60 amperes per sq. ft. of cathode surface with a solution containing 4% to 6% of sulphuric acid for a period of ten minutes will ordinarily deposit some 0.38 ounces of zinc per sq. ft. while under similar conditions the application of the current for fifteen minutes will deposit a considerably greater amount as from 0.50 to 0.7 ounces per sq. ft. depending upon the efficiency of the current, but these amounts will necessarily vary in accordance with different operative conditions.

As the passage of the current from the insoluble anodes to the iron or steel cathodes in the strike coating and operating cells results in the deposition on their respective cathodes, that is, the articles to be coated which act as such, of metallic zinc derived from the solution in the cells and the generation of a chemically equivalent quantity of sulphuric acid, it is thus requisite in order to maintain the solution in the cells at constant acidity to continuously withdraw from each of them a definite volume of the acid solution and to replace it with a corresponding volume of the primary neutral zinc sulfate solution, a result which can be practically effected by feeding into one end of each cell a definite volume of the primary solution and permitting the acid solution from the cell to overflow at the other end, a smaller volume of the primary solution being required to maintain a higher acidity in the cell and a larger volume to maintain a lower acidity for the same rate of acid generation. In accordance with the preferred practice of our invention the effluent solution or overflow from the strike coating cell is directed into the operating cell and as it is of lower acidity than the solution in the latter it to some extent tends to decrease the

acidity thereof while simultaneously a sufficient quantity of the primary solution is also fed to the operating cell so as to hold its acidity substantially constant, and the effluent acid solution from this cell returned to the leaching tank or other point where the leaching operation is performed for the purpose of leaching additional zinc calcine. As the amount of acid contained in this effluent solution is the substantial chemical equivalent of the weight of zinc which has been deposited, a given quantity of the solution when so returned to the leaching operation will, for practical purposes, dissolve from the calcines or other source of zinc supply a weight of zinc equivalent to that which was deposited while that quantity of the effluent solution was being discharged from the operating cell so that the method is thus capable of being carried on uninterruptedly after being once put into operation so long as sufficient zinc calcines or other zinciferous materials are supplied to compensate for the zinc deposited on the iron or steel articles which, from time to time as they receive their coatings of metallic zinc to the required thickness, are removed from the operating cells and after rinsing and drying may be marketed without further treatment.

In the preferred practice of our method as above described raw zinc concentrates are employed as the source of the zinc to be ultimately plated on the ferrous articles and, as heretofore pointed out, it is thus possible by the use of the method to effect a direct transference of the zinc in the ore to the articles and thereby avoid the disadvantages necessarily inherent in first recovering the zinc as a metal by the retort or electrolytic process and then utilizing this metal for hot dipping or electroplating. However, under some conditions it may be preferred to utilize metallic zinc derived in any suitable way instead of zinc calcines in the leaching tank and to there subject this metallic zinc, in a suitable state of division to facilitate rapid dissolving, to the action of the effluent acid solution drawn from the operating cell as hitherto described and in this manner provide the primary neutral zinc sulfate solution for the strike and operating cells. Under these conditions the classifier, ball mill, Dorr thickener and continuous section filter shown on the flow sheet would ordinarily be unnecessary; equally so, if the metallic zinc supplied is devoid of cadmium, copper and/or other impurities, the addition of the zinc dust or other step designed to effect precipitation thereof may be omitted.

While under most conditions but a single operating cell, or a plurality of operating cells each containing zinc sulfate solution of substantially similar acidity and operating at the same current density are employed, it

is within the scope of the invention to utilize a series of operating cells containing solutions of different degrees of acidity and/or operated with currents of varying density.

- 5 Additionally, while we prefer to gradually and continuously feed to the strike coating cell sufficient zinc sulfate solution to maintain the solution in the cell at a constant degree of acidity and to conduct the effluent acid solution displaced by the neutral zinc sulfate solution either to the operating cell or directly back to the leaching tank, it is also within the scope of our invention to refrain from feeding any zinc sulfate solution 10 to the strike coating cell and to permit the acidity of its solution to gradually increase as the strike current is intermittently carried therethrough and to vary the density of this current in accordance with the increasing 15 acidity of the cell instead of operating with a strike current of constant density as hitherto described.

Under certain circumstances it may be deemed advantageous to utilize but a single 20 plating cell instead of separate strike and operating cells and to initially employ in this cell a relatively low acid solution as, for example, one containing 4% or 5% of sulphuric acid so that a strike or initial coating 25 can be formed on the ferrous article in that cell with high current efficiency by momentarily passing a current of relatively high density as, for example, 150 amperes per sq. ft. of cathode surface, the operation 30 in this case being similar to that employed in forming the strike coating in accordance with the preferred practice of the invention. Following the formation of the strike coating, however, instead of transferring the article 35 to another cell having a bath of higher acidity and then continuing the formation of the coating therein by the use of a current of relatively lower density, the article may be allowed to remain in the bath and the 40 passage of the current continued, its amperage, however, being gradually reduced in correspondence with the increasing acidity of the bath until a coating of the desired thickness is obtained. In this manner we are 45 able to form a satisfactory coating by the use of a relatively high acid solution, insoluble anodes and currents of high density with good current efficiency and thus attain, in so far as the character of the ultimate coating 50 is concerned, the results contemplated by our invention, but we do not consider this method of operation as advantageous as the preferred practice of the invention to which we have hitherto referred for the reasons, 55 among others, it is ordinarily less economical and does not lend itself as readily to the desirable cyclic method of operation.

It will of course be understood that the instrumentalities employed in the practice 60 of our improved method may be of any de-

sired form suitable for the performance of their various functions.

In the light of the foregoing disclosure of our invention the advantages arising therefrom and to some of which brief reference has already been made can now more readily be appreciated and may in part be summarized as (a) reduction in plant installation and operating costs and in reduction of fixed charges because of ability to utilize current carrying appliances of relatively small size and capacity; (b) increased operating efficiency of the currents employed due largely to the shortening of the period of hydrogen evolution during the formation of the primary or initial coating of zinc; (c) almost instantaneous coating of the ferrous article with a strike coating of zinc so that but a negligible quantity of the iron or steel is dissolved in the electrolyte before the article is protected from the action of the latter; (d) the strike or incipient coating formed in the strike coating cell upon the article greatly facilitates subsequent coating thereof in the operating cell at economical current density and solution acidity; (e) the ability to employ a relatively low acid solution for the formation of the initial coating which in itself tends to diminish the evolution of hydrogen and decreases tendency of the solution to attack the iron or steel article during the short interval before the initial coating is fully formed; (f) the ability to produce a strongly adherent zinc plating of desired thickness on an iron or steel article by means of relatively high acid solutions of zinc sulfate and currents of such character as may be handled economically within time intervals satisfactory for commercial work; (g) the character of the plating produced, exhibiting as it does substantial chemical purity, an extremely fine crystalline structure, great density, good color and appearance, lack of porosity or sponginess, and particularly markedly greater resistance to corrosion in the presence of weak acids than the zinc coatings which it has hitherto been possible to produce upon iron or steel articles of commerce by any process or method known to us.

Having thus described our invention, we claim and desire to protect by Letters Patent of the United States:

1. In a method of electroplating zinc on iron or steel, the steps of forming a thin initial coating of zinc on the article to be plated by passing thereto from an insoluble anode through a bath of a solution of zinc sulfate of relatively low acidity a direct current of relatively high current density and then after the formation of said initial coating continuing the formation of the plating by the passage of a current of lower density to the article from an insoluble anode through a bath of higher acidity than the first mentioned bath.

2. In a method of electroplating zinc on iron or steel, the steps of forming a thin initial coating of zinc on the article to be plated by passing thereto from an insoluble anode through a bath of a solution of zinc sulfate containing at least 4% of sulphuric acid a direct current of relatively high current density, transferring the initially coated article to another bath containing a solution of zinc sulfate of greater acidity, and then continuing the plating of zinc on the article therein by passing through the second bath from an insoluble anode to the article a direct current of lower density than the first mentioned current. 15
3. In a method of electroplating zinc on iron or steel articles, the steps of electrolyzing a bath of zinc sulfate containing a relatively small amount of sulphuric acid by passing therethrough from an insoluble anode to the article acting as a cathode a current of relatively high density to thereby form on the article an initial relatively thin coating of zinc without excessive hydrogen evolution and then continuing the formation of the coating by electrolyzing a bath of relatively greater acidity by passing therethrough for a longer period a current of relatively lower density from an insoluble anode 30 to the article acting as a cathode.
4. In a method of electroplating zinc on iron or steel articles, the steps of electrolyzing a bath of zinc sulfate containing a relatively small amount of sulphuric acid by passing therethrough from an insoluble anode to the article acting as a cathode a direct current of relatively high density to thereby form on the article an initial relatively thin coating of zinc without excessive hydrogen evolution, then continuing the formation of the coating by electrolyzing a bath of relatively greater acidity by passing therethrough for a longer period a direct current of relatively lower density from an insoluble anode to the article 45 acting as a cathode, and maintaining the acidity of said baths substantially constant by feeding thereto regulated quantities of a neutral solution of zinc sulfate.
5. In a method of electroplating zinc on iron or steel articles, the steps of forming a relatively thin initial coating of zinc on the article by electrolyzing for a short interval a solution of zinc sulfate relatively low in acid by passing a current of relatively high density through the solution from an insoluble anode to the article acting as a cathode, transferring the article after the formation of said initial coating to a second solution of zinc sulfate of greater acidity and continuing the formation of the coating on the article 60 therein by passing through said solution from an insoluble anode to the article acting as a cathode a current of less density for so long a time as may be required to form a coating of the desired thickness on the article and
- maintaining the acidity of said second solution constant by feeding thereto a predetermined regulated quantity of a neutral solution of zinc sulfate.
6. In a method of electroplating zinc on iron or steel articles, the steps of forming an initial relatively thin coating of zinc on the article by electrolyzing a solution of zinc sulfate containing substantially 5% of sulphuric acid by momentarily passing therethrough from an insoluble anode to the article acting as a cathode a direct current having a density of substantially 150 amperes per sq. ft. of cathode surface, then transferring the article to a second solution of zinc sulfate containing substantially 10% of sulphuric acid, continuing the formation of the zinc on the article therein by electrolyzing said solution by passing therethrough from an insoluble anode to the article acting as a cathode a direct current having a density of substantially 60 amperes per sq. ft. of cathode surface and maintaining the acidity of the said solutions substantially constant by feeding thereto sufficient neutral solution of zinc sulfate to compensate for the sulphuric acid generated therein by the passage of the currents. 70
7. In a method of electroplating zinc on iron or steel articles, the steps of forming an initial relatively thin coating of zinc on the article by electrolyzing a solution of zinc sulfate containing substantially 5% of sulphuric acid by momentarily passing therethrough from an insoluble anode to the article acting as a cathode a direct current having a density of substantially 150 amperes per sq. ft. of cathode surface, then transferring the article to a second solution of zinc sulfate containing substantially 10% of sulphuric acid, and continuing the formation of the zinc on the article therein by electrolyzing said solution by passing therethrough from an insoluble anode to the article acting as a cathode a direct current having a density of substantially 60 amperes per sq. ft. of cathode surface. 75
- In witness whereof we have affixed our signatures.
- 115
- SIDNEY H. DAVIS.  
CARL O. ANDERSON.  
WILLIAM N. SMITH.  
HERBERT R. HANLEY.
- 120
- 125
- 130